# EUROPEAN PATENT SPECIFICATION

(11) **EP 2 166 260 B1**
(45) Date of publication and mention of the grant of the patent: **06.06.2012**
(21) Application number: 09010929.9
(22) Date of filing: 26.08.2009
(51) Int. Cl.: F16K 13/10, F17C 1/10, C23F 11/00

(54) **Gas container corrosion protection**
Korrosionsschutz für einen Gasbehälter
Protection contre la corrosion d'un récipient de gaz

(30) Priority: 27.08.2008 GB 0815476
(43) Date of publication of application: 24.03.2010
(73) Proprietor: NGRID Intellectual Property Limited, London WC2N 5EH (GB)
(72) Inventor: Williams, Mark Stephen, London WC2N 5EH (GB)
(74) Representative: Reynolds, Julian David

(56) References cited:
- DE-A1- 3 008 387
- FR-A- 1 077 734
- GB-A- 2 017 831
- JP-A- 59 046 113
- US-A- 2 243 096

## Description

The present invention relates to the storage of gas, and more particularly to techniques for preventing or reducing corrosion in gas containers.

It is well known that certain gases, especially combustible gases for domestic or industrial use, and other volatile gases, need to be safely and securely stored, typically by means of traditional bell holders or enlargeable metal gas holder (hereafter "gas holders") that use a liquid such as water to provide seals for containing the gas.

Gas holders are essential to the continuous supply of gas to customers during periods of high demand. There are currently numerous gas holders in deployed, of which many are the water-sealed type. These operate in a harsh environment, involving raising from and lowering into a tank of water twice a day for the majority of the year, as they are filled and emptied.

The gas holders are conventionally maintained by stripping the existing multi layer paint system and reapplying when required with a similar multi coat paint system. The normal life of the anti-corrosive paint system is ten to fifteen years.

A problem with known systems is that the water based seals, in which a part of a (substantially cylindrical) upper container is in contact with water, are subject to corrosion and need to undergo frequent maintenance, which includes removing and reapplying an anticorrosion coating.

A conventional water-sealed type gas holder 2, and the process for maintenance, is depicted in Figs 1-4 (PRIOR ART). Te holder 2 comprises a base section 4 and two upper sections 6, 8. At the two horizontal rings 10, 12 of the holder 2 are disposed liquid (water) seals (not shown). The typical process for the painting of the gas holder 2 with anti-corrosive paint is as follows.
1. Set up site - Average job duration 16 to 26 weeks.
2. Remove majority of existing coating using high pressure (HP) or ultra high pressure (UHP) water jetting equipment 14.
3. Collect removed coating on netting for disposal as special waste.
4. Degrease holder surface with detergent wash to produce bare metal surface 16.
5. Apply one coat of primer (two-pack epoxy aluminium).
6. Apply two coats of finish (water borne vinyl acrylic).

The process is repeated for each of two horizontal rings 10, 12 of the holder 2. A Mobile Elevated Working Platform (MEWP) or scaffold is required to work at height on the rings 10, 12.

In conventional methods, problems associated with *preparation* include -
- Containment and removal of high volumes of special waste, e.g. removed coating materials plus debris netting, used Personal Protective Equipment (PPE) (disposable).
- Potential noise pollution during surface preparation - HP and UHP jetting units, compressors, site generators, MEWPs etc.
- High level of personnel "health and safety" control measures - PPE for UHP and HP equipment use, noise controls, special waste procedures, waste confinement (screening), collection (keeping debris netting in place and emptying), storage (bunding, security) and inhalation.
- Time consuming, i.e. depending on condition of existing paint and size of holder 2, between one and five days for 2 horizontal plate rings 10, 12.

In conventional methods, problems associated with *coating* include -
- Multiple coats of different materials require
   o Manual application spray, brush application;
   o Large volume to transport and store (on site with bunding);
   o Long process to apply all coats (e.g. Usually prep 2 rings, degrease and allow to dry, prime and allow to cure, apply first finish coat allow to cure, allow second finish coat, allow to cure, raise holder then repeat cycle. Typically there is a minimum of 4 days per two rings of plates (working from ground).
- The two-pack epoxy primer becomes waste if not used in pot life. Material has limited use time before it cures. If paint is mixed and it rains or any is left at the end of a shift, this goes into the waste stream.
- Restrictive weather and temperature tolerance. Materials have upper and lower temperature limits and maximum humidity levels for application that require stringent monitoring

In conventional methods, problems associated with *performance* include -
- Coating breakdown affects surrounding area. Any breakdown in the coating system will allow tank/rain water to penetrate underneath the surrounding coating, causing disbonding of sheets of material. See Fig. 2.
- Maintenance repairs require full surface preparation and reapplication of all coating layers. Areas surrounding damaged require preparation to remove all potentially disbonded material. The full paint system then needs to be applied, involving multiple curing times. It is not adequate to overcoat what's already there. There is potential for hidden areas of coating breakdown. A high degree of preparation for key is a requisite.
- Varying rate of deterioration of the paint system this is affected by localised and prevailing conditions (salt water/winds), original design and material specification of holder 2.

It is known to replace the water seal' of a gas holder with an alternative 'seal' that is not exposed to atmosphere. Such techniques fail to provide an anti-corrosion coating on to the gas holder by use of the existing 'water seal'.

It is also known in certain (non-maintenance) contexts to try to eliminate tank corrosion immediately in contact with the water seal by eliminating oxygen from the seal, or to reduce water vapours from entering the stored gas. (This was important when gas was manufactured locally.) Such techniques fail to provide an alternative to original painting methods. The present Invention seeks to provide a complete anti-corrosion protection to the whole gas holder side sheeting whilst at the same time including (optionally) a colour pigment to enhance the appearance of the gas holder to suit local aesthetics, i.e. an alternative 'painting' system.

JP-A-59046113 discloses a sealing method for a gas treating apparatus, in which part of the recirculated water is withdrawn from the emitting side of a recirculation pump 11 in order to adjust the pH and the solid content of said recirculated water and the liquid withdrawn is supplied to a solid-liquid separator 14 to separate and remove solid components such as fly ash, an adsorbent powder or the like while the solid components after separation ere discharged out of the system and the liquid is sent to a pH adjusting tank 15. The liquid in the pH adjusting tank 15 is neutralized by an alkali solution corresponding to the acidic gas dissolved in sealing water from exhaust gas O to return the pH to neutral and, herein, moisture and steam discharged out of system along with the solid components separated by the solid-liquid separator 14 are replenished. Because the sealing water made neutral in the pH adjusting tank 15 can be repeatedly used, it is returned to a sealing water holding tank 10.

JP-A-48015330 discloses a water-seal type gas holder in which an anti-corrosive agent is added to the sealing water 2, and a sealing water cutoff phase/layer 4 (having a specific gravity lower than that of the sealing water 2 and higher than that of pure water) is formed on the sealing water 4, so that the latter is completely cut off from the outside air. Thus, rainwater is kept out by oil phase 4 and forms a water phase 5 on the oil phase 4. This assists in keeping the amount of sealing water 2 constant. The sealing water cutoff phase 4 may comprise an "oily substance".

The present invention seeks to address the aforementioned and other issues, and provide improved techniques for storage of gases.

According to one aspect of the present invention there is provided a gas container according to claims 1 of the appended claims.

Preferably, the second section has a second anti-corrosion coating on at least a portion thereof. Preferably, the first anti-corrosion coating is caused to be applied to at least a part of said second anti-corrosion coating,

In one embodiment, the gas container comprises a number of further sections configured in a telescopic arrangement, whereby the volume of the gas container is variable; and wherein one of said liquid seals is provided between adjacent sections. Preferably, the first and/or further second sections have the second anti-corrosion coating on at least a portion thereof.

Preferably, the second anti-corrosion coating comprises a cured coating applied by painting or spraying. Preferably, the first anti-corrosion coating comprises a floatable anti-corrosion coating, e.g. Floatcoat (RTM).

According to another aspect of the present invention there is provided a method of assembling a gas container, according to claims 6 of the appended claims.

Preferably, the second section has a second anti-corrosion coating on at least a portion thereof. Preferably, the first anti-corrosion coating is caused to be applied to at least a part of said second anti-corrosion coating.

In one embodiment, the there are provided a number of further sections configured In a telescopic arrangement, whereby the volume of the gas container is variable; and wherein one of said liquid seals is provided between adjacent sections. Preferably, the first and/or further second sections have the second anti-corrosion coating on at least a portion thereof.

Preferably, the second anti-corrosion coating comprises a cured coating applied by painting or spraying.

Preferably, the first anti-corrosion coating comprises a floatable anti-corrosion coating, e.g. Floatcoat (RTM).

According to another aspect of the present invention there is provided a method of maintaining a gas container, according to claims 11 of the appended claims.

Preferably, the second section has a second anti-corrosion coating on at least a portion thereof. Preferably, the first anti-corrosion coating Is caused to be applied to at least a part of said second anti-corrosion coating.

In one embodiment, the gas container comprises a number of further sections configured in a telescopic arrangement, whereby the volume of the gas container is variable; and wherein one of said liquid seals is provided between adjacent sections. Preferably, the first and/or further second sections have the second anti-corrosion coating on at least a portion thereof.

Preferably, the second anti-corrosion coating comprises a cured coating applied by painting or spraying. Preferably, the first anti-corrosion coating comprises a floatable anti-corrosion coating, e.g. Floatcoat (RTM).

The techniques according to the invention move away from multiple paint layers to a 'self healing' two-coat system that is much healthier, quicker and easier to apply and maintain.

The first application requires a similar level of surface preparation as conventional painting to remove the existing coating materials. This high level of preparation is not required for future maintenance coatings. The first coat material is roller applied to the prepared surface of the gas holder to a thickness of, for example, about 100 microns. This coat is allowed to cure fully after completion prior to the final coating material being used.

The second coat material does not require manual application to the holder surface it is "floated" on the water surface of the gas holder seals and adheres to the surface as the holder is raised and lowered. This second coat is a non setting gel type material which, once adhered, remains on the holder surface to protect it from corrosion.

Advantages of the invention include -
- No risk to human health or the environment. The invention has many health, safety and environmental benefits for the workforce and the local community.
- Application is extremely tolerant to adverse weather / temperatures.
- Trials show excellent corrosion protection achieved through a single application. Average job duration 8 to 13 weeks.

Further advantages of the invention in relation to *Safety and Health* include -
- Only one roller applied coat. Only a single coat requires manual application, reducing the physical effort and time of application by a factor of three over the conventional method
- Second coat applied from holder tank and cups. The second material effectively apples itself as the holder is raised and lowered.
- Less material required reducing manual handling and use of portable plant.
- The process reduces health hazards and noise exposure.
- No repeat preparation required in subsequent years. Removal of the need for high specification surface preparation for future applications significantly reduces health hazards and noise exposure for operatives and the local community.

Further advantages of the invention in relation to *Environment* include -
- System is "Self Healing" requires minimal maintenance repairs. Any areas of mechanical damage to the coatings will re-coat with the second non setting material and prevent corrosion.
- No subsequent stripping of degraded paint film, reducing future waste generation.
- Significant reduction in material usage, reducing manual handling and the carbon footprint for transportation and application.
- Material is environmentally friendly.
- Job durations reduced.

It has been found that the Invention provides a 50% saving compared with conventional maintenance painting costs. There is an estimated 75% saving in future maintenance coating costs where the initial high standard of preparation will not be required.

Embodiments of the invention will now be described in detail, by way of example, with reference to the accompanying drawings, in which:
Figures 1 to 4 (PRIOR ART) show a conventional gas holder and known techniques for maintenance;
Figure 5 shows schematically in cross-section a gas holder and techniques for maintenance, according to a first embodiment of the invention, (a) complete view showing movable sections, and (b) a liquid sealing ring in detail; and
Figure 6 shows a gas holder and techniques for maintenance, according to a second embodiment of the invention, (a) complete view showing movable sections, and (b) schematically in cross-section showing liquid sealing in detail.

In the description and drawings, like numerals are used to designate like elements. Unless indicated otherwise, any individual design features and components may be used in combination with any other design features and components disclosed herein.

Figure 5(a) shows schematically in cross-section a gas holder and techniques for maintenance, according to a first embodiment of the invention, in complete view showing movable sections. The construction of the gas holder 2 is the same as in Figs 1 to 4, except as described below. In the is case, as well as base section 4, there are four upper sections 6, 8, 9 and 11, having associated rings (liquid seals) 10, 12, 13. The upper section 11 has a dome 15. Each section 6, 8, 9, 11 is capable of containing a substantial quantity of gas, and the each section is constructed an arranged so as to be movable vertically in telescopic fashion in relation to an adjacent section, dependent on the amount of gas stored or to be stored in the gas holder 2.

Figure 5(b) shows a liquid sealing ring 10 in more detail. For each of the sections, including sections 6 and 8, there is optionally but preferably provided a first anti-corrosion coating as described above in the process described with reference to Figs 1 to 4, i.e. one coat of primer (two-pack epoxy aluminium), followed by two coats of finish (water borne vinyl acrylic). Suitably, the first anti-corrosion coating comprises a coating available under the trade name Performance 105. This is suitably applied by roller. In this embodiment, within the ring 10 a liquid seal 18 is provided by a reservoir of water 20 in which an upper limb 21 of section 6 is immersed. The upper limb is movable vertically in relation to the water 20 during increases and decreases in the volume of the gas holder 2.

According to the invention, an anti-corrosion coating 22 is provided. The anti-corrosion coating 22 comprises a material that will float on the water 20, and is suitably a floatable anti-corrosion coating available under the trade name Floatcoat (RTM). The anti-corrosion coating 22 is applied from a holder tank and cups (not shown), i.e. all applied at ground/tank level from an applicator (not shown). This can be achieved in 1 day for all 3 sections in a typical installation.

In this embodiment, water is used as the liquid seal.

In this embodiment, Floatcoat (RTM) is used as the anti-corrosion coating 22; however, it will be appreciated by persons skilled in the art that other liquids may be used. The requirement is only that the anti-corrosion coating 22 has a lower density than the liquid (water), so as to float thereon. Suitably, the anti-corrosion coating 22 comprises an organic composition containing a corrosion inhibitor. Suitably, the organic composition is a naphthenic mineral oil based composition.

Figure 6 shows a gas holder 602 and techniques for maintenance, according to a second embodiment of the invention, complete view showing movable sections. This is the same as the first embodiment, except as described below. The sections include a base section 604 and upper section 606.

Figure 7 shows schematically in cross-section the construction of the gas holder 602, showing a liquid sealing and the anti-corrosion coating in detail. As shown in Fig. 7(b), a first anti-corrosion coating 608 is optionally applied - this is the same coating as for the first embodiment. The base section 604 is partially filled with water 622 and a suitable quantity of Floatcoat (RTM) added as a second anti-corrosion coating 622 (Fig. 7(c)). In accordance with this embodiment, and as shown in Fig. 7(d), the assembled gas holder 602 provides a space 603 of variable volume for storage of gas.

It will be appreciated by skilled persons that numerous advantages are afforded by the invention and embodiments thereof. Application is extremely tolerant to adverse weather conditions and temperatures. Above freezing, there is no standing ice or risk of same. In humid conditions, there is no standing/surface water.

Trials show excellent corrosion protection achieved through a single application: tests showed no corrosion evident after 2.5 years. The average job duration was 8 to 13 weeks - 50% of duration for conventional painting for first application. Duration for the second recoat is reduced - by preparation time of 1 to 2 weeks per lift (section) and possibly application of Performance 105 by roller.

Less material is required, reducing manual handling and use of portable plant. The details for a comparative test are as follows.
Conventional maintenance method (Figs 1-4): Primer/Finish - 2300 litres.
Techniques according to embodiments of the invention:
- "Performance 105" - 400 litres
- "Floatcoat" (RTM) - 560 litres
- Total 960 litres
i.e. 42% by volume of the materials for the conventional method, excluding any waste materials in conventional application.

The material poses minimum health hazards - requires only standard PPE for application, i.e. inhalation, COSHH (in the UK). The process poses minimum noise exposure - surface preparation is required on first application, however potentially not as stringent. Such noisy preparation is not required for future coatings, thus overall job duration is reduced further. The only requirement is to apply further quantities of the second anti-corrosion coating (e.g. Floatcoat (RTM)).

A further advantage is that the system is "self healing", i.e. it requires minimal maintenance repairs - Mechanical damage to Performance105/Floatcoat does not travel under the surrounding surface. Surplus of the second anti-corrosion coating (e.g. Floatcoat (RTM)) on the tank/cup, or movement of surface Floatcoat (RTM), will 'self Heal" small areas of damage, i.e. carriage wear. Maintenance repair only requires minimum surface clean (degrease) and application of more of the second anti-corrosion coating (e.g. Floatcoat (RTM)).

It will be understood that it is not essential that the Performance 105 coating is applied. Floatcoat (RTM) affords sufficient anti-corrosion protection in its own right; however, an increased level of protection is afforded by utilising the hybrid system, and additionally a colouration can be provided through the Performance 105, which is not possible with Floatcoat (RTM) alone.

## Claims

1. A gas container (2), comprising.
at least 3 first section (4) and a second section (6), the first and second sections (4,6) being substantially hollow and movable relative to each other;
a liquid seal (18) for sealing gas within the container (2), the liquid seal (18) being disposed between the first section (4) and the second section (6);
wherein a first anti-corrorion coating (22; 622) is provided so as to float on the surface of the liquid (20) in said liquid seal; whereby, in use, the first anti-corrosion coaling (22: 622) is caused to be applied to at least a portion of said second section (6) during motion of the second section (6) relative to the first section (4).

2. The gas container of claim 1, wherein the liquid seal (18) comprises a sealing container (10) of cup-shaped cross-section in witch water or a water based liquid (20) is present.

3. The gas container of claim 1 or 2, wherein the second section (6) has a second anti-corrosion coating (608) on at least a portion thereof.

4. The gas container of claim 3, wherein the first anti-corrosion coating (22; 622) is caused to be applied to at least a part of said second anti-corrosion coating (608).

5. The gas container of any of the preceding claims, comprising a number of further sections (8, 9, 11) configured in a telescopic arrangement, whereby the volume of the gas container (2) is variable; and wherein one of said liquid seals (16) is provided between adjacent sections (8, 9, 11).

6. A method of assembling a gas container (2), comprising:
providing a substantially hollow first section (4);
providing a substantially hollow second section (6);
providing a liquid seal (18) for sealing gas within the container, the liquid seal being disposed between the first section (4) and the second section (6);
providing a first anti-corrosion coating (22; 622) so as to float on the surface of liquid (20) in said liquid seal (18);
causing the first and second sections (4, 6) to engage or move relative to each other, whereby the first anti-corrosion coating (22: 622) is caused to be applied to at least a portion of said second section (6), for example during motion of the second section (6) relative to the first section (4),

7. The method of claim 6, wherein the liquid seal (18) comprises a seating container (10) of cup-shaped cross-section in which water or a water based liquid (20) is present.

8. The method of claim 6 or 7, wherein the second section (8) has a second anti-corrosion coating (608) on at least a portion thereof,

9. The method of claim 8, wherein the first anti-corrosion coating (22; 622) is caused to be applied to at least a part of said second anti-corrosion coating (608).

10. The method of any of claims 8 to 9, comprising a number of further sections (8, 9, 11) configured in a telescopic arrangement, whereby the volume of the gas container (2) is variable: and wherein one of said liquid seals (18) is provided between adjacent sections.

11. A method of maintaining a gas container (2), the container comprising a first section (4) and a second section (6), the first and second sections (4, 6) being substantially hollow and movable relative to each other; a liquid seal (18) being provided for sealing gas within the container (2), the liquid seal being disposed between the first section (4) and the second section (6), the method comprising:
providing a first anti-corrosion coating (22; 622) so as to float on the surface of the liquid (20) of said liquid seal (18),
causing the first and second sections (4, 6) to engage or move relative to each other, whereby the first anti-corrosion coating (22; 622) is caused to be applied to at least a portion of said second section (6), for example during motion of the second section (6) relative to the first section (4).

12. The method of claim 11, wherein the liquid seal comprises a sealing container (10) of cup-shaped cross-section in which water or a water based liquid (20) is present.

13. The method of claim 11 or 12, wherein the second section (6) has a second anti-corrosion coating (608) on at least a portion thereof.

14. The method of claim 13, wherein the first anti-corrosion coating (22; 822) is caused to be applied to at least a part of said second anti-corrosion coating (608).

15. The method of any of claims 11 to 14, comprising a number of further sections (8, 9, 11) configured in a telescopic arrangement, whereby the volume of the gas container (2) is variable; and wherein one of said liquid seals (18) is provided between adjacent sections.

## Patentansprüche

1. Gasbehälter (2), umfassend
zumindest einen ersten Abschnitt (4) und einen zweiten Abschnitt (6), wobei der erste und der zweite Abschnitt (4, 6) im Wesentlichen hohl und in Bezug zueinander beweglich sind;
eine Flüssigkeitsdichtung (18) zum Einschließen von Gas innerhalb des Behälters (2), wobei die Flüssigkeitsdichtung (18) zwischen dem ersten Abschnitt (4) und dem zweiten Abschnitt (6) angeordnet ist;
wobei eine erste Antikorrosionsbeschichtung (22; 622) so vorgesehen ist, dass sie auf der Oberfläche der Flüssigkeit (20) in den Flüssigkeitsdichtungen schwimmt; wodurch, bei Verwendung, bewirkt wird, dass die erste Antikorrosionsbeschichtung (22; 622) auf zumindest einen Teil des zweiten Abschnitts (6) während der Bewegung des zweiten Abschnitts (6) in Bezug auf den ersten Abschnitt (4) aufgebracht wird.

2. Gasbehälter nach Anspruch 1, wobei die Flüssigkeitsdichtung (18) einen Dichtungsbehälter (10) mit becherförmigem Querschnitt umfasst, in dem Wasser oder eine wasserbasierte Flüssigkeit (20) vorhanden ist.

3. Gasbehälter nach Anspruch 1 oder 2, wobei der zweite Abschnitt (6) eine zweite Antikorrosionsbeschichtung (608) auf zumindest einem Teil desselben aufweist.

4. Gasbehälter nach Anspruch 3, wobei bewirkt wird, dass die erste Antikorrosionsbeschichtung (22; 622) auf zumindest einen Teil der zweiten Antikorrosionsbeschichtung (608) aufgebracht wird.

5. Gasbehälter nach einem der vorstehenden Ansprüche, der eine Anzahl weiterer Abschnitte (8, 9, 11) umfasst, die in einer teleskopischen Anordnung ausgebildet sind, wodurch das Volumen des Gasbehälters (2) variabel ist; und wobei eine der Flüssigkeitsdichtungen (18) zwischen benachbarten Abschnitten (8, 9, 11) vorgesehen ist.

6. Verfahren zum Zusammenbauen eines Gasbehälters (2), umfassend:
Bereitstellen eines im Wesentlichen hohlen ersten Abschnitts (4);
Bereitstellen eines im Wesentlichen hohlen zweiten Abschnitts (6);
Bereitstellen einer Flüssigkeitsdichtung (18) zum Einschließen von Gas innerhalb des Behälters, wobei die Flüssigkeitsdichtung zwischen dem ersten Abschnitt (4) und dem zweiten Abschnitt (6) angeordnet wird;
Bereitstellen einer ersten Antikorrosionsbeschichtung (22; 622) so, dass sie auf der Oberfläche der Flüssigkeit (20) in den Flüssigkeitsdichtungen (18) schwimmt;
Bewirken, dass der erste und der zweite Abschnitt (4, 6) in Eingriff gelangen oder sich in Bezug zueinander bewegen, wodurch bewirkt wird, dass die erste Antikorrosionsbeschichtung (22; 622) auf zumindest einen Teil des zweiten Abschnitts (6) aufgebracht wird, beispielsweise während der Bewegung des zweiten Abschnitts (6) in Bezug auf den ersten Abschnitt (4).

7. Verfahren nach Anspruch 6, wobei die Flüssigkeitsdichtung (18) einen Dichtungsbehälter (10) mit becherförmigem Querschnitt umfasst, in dem Wasser oder eine wasserbasierte Flüssigkeit (20) vorhanden ist.

8. Verfahren nach Anspruch 6 oder 7, wobei der zweite Abschnitt (6) eine zweite Antikorrosionsbeschichtung (608) auf zumindest einem Teil desselben aufweist.

9. Verfahren nach Anspruch 8, wobei bewirkt wird, dass die erste Antikorrosionsbeschichtung (22; 622) auf zumindest einen Teil der zweiten Antikorrosionsbeschichtung (608) aufgebracht wird.

10. Verfahren nach einem der Ansprüche 6 bis 9, das eine Anzahl weiterer Abschnitte (8, 9, 11) umfasst, die in einer teleskopischen Anordnung ausgebildet werden, wodurch das Volumen des Gasbehälters (2) variabel ist; und wobei eine der Flüssigkeitsdichtungen (18) zwischen benachbarten Abschnitten vorgesehen ist.

11. Verfahren zum Instandhalten eines Gasbehälters (2), der Behälter umfassend einen ersten Abschnitt (4) und einen zweiten Abschnitt (6), wobei der erste und der zweite Abschnitt (4, 6) im Wesentlichen hohl und in Bezug zueinander beweglich sind; eine Flüssigkeitsdichtung (18), die zum Einschließen von Gas innerhalb des Behälters (2) vorgesehen ist, wobei die Flüssigkeitsdichtung zwischen dem ersten Abschnitt (4) und dem zweiten Abschnitt (6) angeordnet ist, das Verfahren umfassend:
Bereitstellen einer ersten Antikorrosionsbeschichtung (22; 622) so, dass sie auf der Oberfläche der Flüssigkeit (20) der Flüssigkeitsdichtungen (18) schwimmt,
Bewirken, dass der erste und der zweite Abschnitt (4, 6) in Eingriff gelangen oder sich in Bezug zueinander bewegen, wodurch bewirkt wird, dass die erste Antikorrosionsbeschichtung (22; 622) auf zumindest einen Teil des zweiten Abschnitts (6) aufgetragen wird, beispielsweise während der Bewegung des zweiten Abschnitts (6) in Bezug auf den ersten Abschnitt (4).

12. Verfahren nach Anspruch 11, wobei die Flüssigkeitsdichtung einen Dichtungsbehälter (10) mit becherförmigem Querschnitt umfasst, in dem Wasser oder eine wasserbasierte Flüssigkeit (20) vorhanden ist.

13. Verfahren nach Anspruch 11 oder 12, wobei der zweite Abschnitt (6) eine zweite Antikorrosionsbeschichtung (608) auf zumindest einem Teil desselben aufweist.

14. Verfahren nach Anspruch 13, wobei bewirkt wird, dass die erste Antikorrosionsbeschichtung (22; 622) auf zumindest einen Teil der zweiten Antikorrosionsbeschichtung (608) aufgebracht wird.

15. Verfahren nach einem der Ansprüche 11 bis 14, das eine Anzahl weiterer Abschnitte (8, 9, 11) umfasst, die in einer teleskopischen Anordnung ausgebildet sind, wodurch das Volumen des Gasbehälters (2) variabel ist; und wobei eine der Flüssigkeitsdichtungen (18) zwischen benachbarten Abschnitten vorgesehen ist.

## Revendications

1. Récipient de gaz (2), comprenant :
au moins une première section (4) et une seconde section (6), les première et seconde sections (4, 6) étant sensiblement creuses et mobiles l'une par rapport à l'autre ;
un joint liquide (18) destiné à assurer l'hermétisation vis-à-vis du gaz contenu dans le récipient (2), le joint liquide (18) étant disposé entre la première section (4) et la seconde section (6) ;
dans lequel un premier revêtement anti-corrosion (22 ; 622) est prévu de manière à flotter à la surface du liquide (20) dans lesdits joints liquides, moyennant quoi, à l'usage, le premier revêtement anti-corrosion (22 ; 622) est amené à s'appliquer sur au moins une partie de ladite seconde section (6) pendant le mouvement de la seconde section (6) par rapport à la première section (4).

2. Récipient de gaz selon la revendication 1, dans lequel le joint liquide (18) comprennent un récipient d'hermétisation (10) de section transversale en forme de coupelle dans lequel se trouve de l'eau ou un liquide à base d'eau (20).

3. Récipient de gaz selon la revendication 1 ou 2, dans lequel la seconde section (6) présente un second revêtement anti-corrosion (608) sur au moins une partie de celle-ci.

4. Récipient de gaz selon la revendication 3, dans lequel le premier revêtement anti-corrosion (22 ; 622) est amené à s'appliquer sur au moins une partie dudit second revêtement anti-corrosion (608).

5. Récipient de gaz selon l'une quelconque des revendications précédentes, comprenant un certain nombre de sections supplémentaires (8, 9, 11) configurées selon un agencement télescopique, moyennant lesquelles le volume du récipient de gaz (2) est susceptible de varier ; et dans lequel l'un desdits joints liquides (18) est prévu entre des sections (8, 9, 11) adjacentes.

6. Procédé d'assemblage d'un récipient de gaz (2), comprenant :
la mise à disposition d'une première section (4) sensiblement creuse ;
la mise à disposition d'une seconde section (6) sensiblement creuse ;
la mise à disposition d'un joint liquide (18) destiné à assurer l'hermétisation vis-à-vis du gaz contenu dans le récipient, le joint liquide étant disposé entre la première section (4) et la seconde section (6) ;
la mise à disposition d'un premier revêtement anti-corrosion (22 ; 622) de manière à ce que celui-ci flotte à la surface du liquide (20) desdits joints liquides (18) ;
l'emboîtement ou le mouvement l'une par rapport à l'autre des première et seconde sections (4, 6), moyennant quoi le premier revêtement anti-corrosion (22 ; 622) est amené à s'appliquer sur au moins une partie de ladite seconde section (6), par exemple pendant le mouvement de la seconde section (6) par rapport à la première section (4).

7. Procédé selon la revendication 6, dans lequel le joint liquide (18) comprennent un récipient d'hermétisation (10) de section transversale en forme de coupelle dans lequel se trouve de l'eau ou un liquide à base d'eau (20).

8. Procédé selon la revendication 6 ou 7, dans lequel la seconde section (6) présente un second revêtement anti-corrosion (608) sur au moins une partie de celle-ci.

9. Procédé selon la revendication 8, dans lequel le premier revêtement anti-corrosion (22 ; 622) est amené à s'appliquer sur au moins une partie dudit second revêtement anti-corrosion (608).

10. Procédé selon l'une quelconque des revendications 6 à 9, comprenant un certain nombre de sections supplémentaires (8, 9, 11) configurées selon un agencement télescopique, moyennant lesquelles le volume du récipient de gaz (2) est susceptible de varier ; et dans lequel l'un desdits joints liquides (18) est prévu entre des sections adjacentes.

11. Procédé d'entretien d'un récipient de gaz (2), le récipient comprenant une première section (4) et une seconde section (6), les première et seconde sections (4, 6) étant sensiblement creuses et mobiles l'une par rapport à l'autre ; un joint liquide (18) étant prévu pour assurer l'hermétisation vis-à-vis du gaz contenu dans le récipient (2), le joint liquide étant disposé entre la première section (4) et la seconde section (6), le procédé comprenant :
la mise à disposition d'un premier revêtement anti-corrosion (22 ; 622) de manière que celui-ci flotte à la surface du liquide (20) desdits joints liquides (18) ;
l'emboîtement ou le mouvement l'une par rapport à l'autre des première et seconde sections (4, 6), moyennant quoi le premier revêtement anti-corrosion (22 ; 622) est amené à s'appliquer sur au moins une partie de ladite seconde section (6), par exemple pendant le mouvement de la seconde section (6) par rapport à la première section (4).

12. Procédé selon la revendication 11, dans lequel le joint liquide comprennent un récipient d'hermétisation (10) de section transversale en forme de coupelle dans lequel se trouve de l'eau ou un liquide à base d'eau (20).

13. Procédé selon la revendication 11 ou 12, dans lequel la seconde section (6) présente un second revêtement anti-corrosion (608) sur au moins une partie de celle-ci.

14. Procédé selon la revendication 13, dans lequel le premier revêtement anti-corrosion (22 ; 622) est amené à s'appliquer sur au moins une partie dudit second revêtement anti-corrosion (608).

15. Procédé selon l'une quelconque des revendications 11 à 14, comprenant un certain nombre de sections supplémentaires (8, 9, 11) configurées selon un agencement télescopique, moyennant lesquelles le volume du récipient de gaz (2) est susceptible de varier ; et dans lequel l'un desdits joints liquides (18) est prévu entre des sections adjacentes.
